

1

3,042,514

**DIFFUSION-TRANSFER REVERSAL PROCESS**  
 Curt B. Roth, Binghamton, N.Y., assignor to General  
 Aniline & Film Corporation, New York, N.Y., a cor-  
 poration of Delaware  
 No Drawing. Filed Aug. 6, 1959, Ser. No. 831,953  
 23 Claims. (Cl. 96—29)

This invention relates to a novel photographic process. More particularly, this invention relates to a novel diffusion-transfer reversal process wherein ordinary tap water is used as the processing liquid.

The diffusion-transfer reversal process, referred to hereinafter as the DTR process, comprises exposing a photographic element comprising a base having thereon a coating of a light sensitive silver halide emulsion and developing the exposed coating with a developer containing a silver halide solvent while the coating is in contact with a specially-prepared layer which is not light sensitive. In the course of forming a negative image in the exposed coating, the solvent in the developer dissolves the unexposed silver halide which is transferred image-wise to the specially-prepared layer to form thereon a positive image by reaction of the dissolved silver halide with substances present in the layer. The DTR process as heretofore practiced is relatively slow, complicated and difficult to control.

It is an object of this invention to provide a novel diffusion-transfer reversal process which is simple and materially easier and faster in operation than the known DTR processes.

It is a further object of this invention to provide a novel diffusion-transfer process utilizing a commercial print-out emulsion as the photosensitive layer.

It is a still further object of this invention to provide a novel diffusion-transfer process utilizing water for accomplishing the transfer of the image from the photosensitive layer to the receiving layer.

Other objects and advantages of this invention will appear to those skilled in the art from the detailed description thereof given below.

Briefly, the novel process of this invention comprises exposing a photosensitive film comprising a base having as a photosensitive layer a known print-out emulsion and then pressing the exposed film against an image receiving layer in the presence of moisture. The moisture may be supplied by means of ordinary tap water or deionized water. The pressing of the two layers may take place at room temperature. A contact time of from 1-20 seconds, preferably about 2 to 5 seconds is sufficient to accomplish the transfer of the image. The two very slightly moist layers are then separated and dried.

If desired, this process can be practiced as a "dry process." Heat alone may be utilized to accomplish the transfer of the image. A reagent can be added to the coating which loses moisture on heating. Such reagent is disclosed in German Patent No. 888,045 and in Bild und Ton, 11, 62 (1958). The increased temperature may be such as to speed up the diffusion to such an extent that a more rolling of the contacting layers between hot rollers will be sufficient to transfer the image.

If desired, this process can be practiced as a "semi-dry process." The moisture necessary to accomplish the transfer may be supplied in the form of steam. These last named modifications would, for all practical purposes, be dry transfer processes.

Print-out emulsions are well known in the art. These emulsions are described in various publications. Special reference is here made to pages 245-257 of a book by T. T. Baker entitled, "Photographic Emulsion Technique" 1948, published by American Photographic Publishing

2

Company. These emulsions are also described in a book entitled, "Photographic Facts and Formulas" (1947), pages 188-200, by E. J. Wall and in a book entitled, "Chimie Photographique" (1957), pages 299-301, by Pierre Glafkides.

An example of a print-out emulsion composition which is given in the book by Baker is the following:

|                           |     |        |
|---------------------------|-----|--------|
| Ammonium chloride         | g—  | 2.5    |
| Sodium potassium tartrate | g—  | 5.0    |
| Gelatin                   | g—  | 80.0   |
| Silver nitrate            | g—  | 25.0   |
| Citric acid               | g—  | 10.0   |
| Water                     | cc— | 1000.0 |
| Alcohol                   | cc— | 40.0   |

Many variations in both the ingredients and proportions of print-out emulsions are described in the various books referred to above. These emulsions all contain a soluble silver salt such as silver nitrate, for example, a halide, such as ammonium chloride, sodium chloride, etc., capable of reacting with the soluble silver salt to form silver halide, the amount of soluble silver salt in the composition being in excess of that which will react with the halide to form silver halide so that a certain amount of the soluble silver salt is present in the emulsion after exposure. In addition to the aforesaid essential components, such emulsions may also contain various secondary adjuncts such as surfactants, ultraviolet absorbers and the like.

The print-out emulsion may be coated on any desired base used in the photographic art. Among the suitable bases are the cellulose esters such as cellulose acetate, cellulose nitrate, for example, the vinyl resins such as vinyl acetate, paper, metals and others.

The image-receiving layer may be baryta subbed paper base as such or the baryta paper may be coated with a layer containing any one or a mixture of the following substances:  $ZnO$ ,  $Mn(OAc)_2$ ,  $ZnO + Mn(OAc)_2$ ,  $TiO_2$ ,  $TiO_2 + Mn(OAc)_2$ , ascorbic acid, colloidal  $ZnS$ , coll.  $CdS$ , colloidal Ag, colloidal sulfur,  $Na_2S$ , 2-mercaptopbenzothiazole, phenyl-mercapto-tetrazole, colloidal silica such as silica aerogel, Santogel, fuller's earth, diatomaceous earth, kieselguhr, wood flour, infusorial earth, bentonite, filter aids such as Celite, Super-Floss and finely-powdered glass, talc, mica and the like.

Upon exposure of the light sensitive layer, photolytic silver is formed in the exposed areas. This photolytic silver does not diffuse. The unexposed areas contain still the soluble silver salts such as silver nitrate, silver citrate and/or silver and ammonia complexes, depending upon the composition of the print-out type emulsion used. Upon contact of the exposed layer with the image receiving layer in the presence of water, the water soluble silver salts dissolve and diffuse into the image-receiving layer to form the image.

The differences between the prior art DTR processes and the novel DTR process of this invention may be summarized as follows:

In the prior art processes, only silver halide is used in the light sensitive emulsion. I use soluble silver salts in my light sensitive emulsion. The prior art processes use a viscous, complicated, unstable paste which must be applied uniformly to form a film of uniform thickness in order to properly develop and transfer the image.

I use only water, which may be ordinary tap water, for this purpose. The prior art process must include a solvent for silver halide in the processing paste. I do not use any silver halide solvent. In fact, I do not need any silver halide at all. It may, sometimes, be desirable to have some silver halides present in the light sensitive layer in order to increase speed or to extend the spectral sensitivity of this layer by optical or chemical sensitiza-

tion. However, the silver halide is no essential ingredient and does not take part in the DTR step. The development and transfer of the prior art processes takes about 60 seconds whereas in my process 3 seconds or less is sufficient. My process may be carried out in the presence of room light whereas the prior art processes must be carried out in darkness.

The following specific examples illustrate my novel process. It is to be understood, however, that these examples are given by of illustration and not by way of limitation.

*Example I*

(1) A light sensitive coating was prepared by adding to a commercial print-out emulsion as obtained from production (50.0 g.) a 20% aqueous formaldehyde solution (1.0 ml.), and coating the above mixture at 40° C. onto a subbed cellulose triacetate film base.

(2) The light sensitive coating was exposed for 5 minutes as follows:

The coating was placed behind a photographic negative in a printing frame. The printing frame was placed 41 cm. from a Medium Beam Reflector Photo Lamp. Between the lamp and the printing frame was placed an 18 cm. wide, parallel-sided battery jar filled with deionized water. The light intensity at the plane, where the printing frame stood during exposure, was set at 200 foot candles. The intensity of the lamp output was controlled by means of a voltage regulator. The light intensity was measured before each exposure with a Weston Foot-Candle Meter, model L-61.

(3) The exposed light sensitive coating was rolled into contact with the image-receiving paper which consisted of baryta subbed paper base through a bath containing tap water for a period of 5 seconds.

The coatings were then stripped apart 5 seconds after they had emerged together from the roller system.

(4) The image on the image-receiving paper was then washed for 1 minute with running (20° C.) tap water.

It was found that:

- (1) Both the exposed and unexposed areas of the light sensitive coating transferred to the image-receiving paper base.
- (2) When washed with cold water, the unexposed background ( $Ag^+$ ) washed almost entirely off, but the exposed letters ( $Ag^{\circ}$ ) did not. Thus, a positive image consisting of dark brown-black letters on a pink background was obtained.

*Example II*

(1) The light sensitive coating was prepared by coating the following mixture (40° C.) on baryta subbed paper base:

Commercial print-out emulsion.....g. 50  
 $MnSO_4 \cdot 4H_2O$  (50% aqueous solution).....ml. 1

(2) The image-receiving coating was prepared by coating the following mixture (40° C.) on baryta subbed paper base:

10% aq. surface gel.....g. 35  
8% aq. Saponin.....ml. 0.5  
"Standard AgI emulsion".....g. 5  
10% aq. formaldehyde.....ml. 0.5

(3) The light sensitive coating was exposed through a photographic positive for 5 minutes in the same setup as described in Example I, step 2.

(4) The exposed light sensitive coating was rolled into contact with the image-receiving coating through a bath containing deionized water for a period of 5 seconds.

The coatings were then stripped apart 5 seconds after they had emerged together from the roller system.

The image-receiving layer was then dipped into 5% aqueous NaOH for 30 seconds, and then washed 1 minute with running 20° C. tap water.

It was found that:

- (1) Almost all of the unexposed and part of the exposed portions of the light sensitive coating transferred to the image-receiving layer.
- (2) A reversal image consisting of dark brown letters on a dark background was obtained.

*Example III*

(1) The light sensitive coating was prepared by coating the following mixture (40° C.) on transparent film base:

|                                          |         |
|------------------------------------------|---------|
| Commercial print-out emulsion.....       | g. 15   |
| "Standard silver chloride emulsion"..... | g. 35   |
| 8% aq. Saponin.....                      | ml. 0.3 |
| 15 10% aq. solution of K-Cr-Alum.....    | ml. 1   |

(2) The image-receiving layer was prepared by pulling strips of baryta subbed paper base through a 2% aqueous solution of ascorbic acid.

(3) The light sensitive coating was exposed through a photographic positive for 7 minutes in the same setup as described in Example I, step 2.

(4) The exposed light sensitive coating was rolled into contact with the image-receiving coating through a bath containing deionized water for a period of 5 seconds.

The coatings were then stripped apart 5 seconds after they had emerged together from the roller system.

It was found that:

- (1) The unexposed letters transferred very nicely from the exposed to the image-receiving layer; very little of the exposed background transferred to the image-receiving layer.
- (2) An acceptable positive image consisting of light-black letters on an off-white background was obtained.
- (3) No washing of the receiving layer is necessary.

*Example IV*

(1) The light sensitive coating used was the same as that described in Example III, step 1.

(2) The image-receiving coating was prepared by pulling strips of baryta subbed paper base through a solution consisting of 30 mg. of 2-mercaptopbenzothiazole per liter of distilled methanol; these strips were dried thoroughly before using.

(3) The light sensitive coating was exposed through a photographic positive for 6 minutes in the same setup as described in Example I, step 2.

(4) The exposed light sensitive coating was rolled into contact with the image-receiving coating through a bath containing tap water for a period of 5 seconds.

The coatings were then stripped apart 5 to 10 seconds after they had emerged together from the bath.

It was found that:

- (1) The unexposed letters of the light sensitive coating transferred satisfactorily to the image-receiving layers; very little of the exposed background transferred.
- (2) A reversal image consisting of red-brown letters on a light-pink background was obtained.

*Example V*

(1) The light sensitive coating used was the same as that described in Example III, step 1.

(2) The image-receiving coating was prepared by pulling strips of baryta subbed paper base through a solution consisting of 30 mg. of phenyl-mercapto-tetrazole per liter of distilled methanol; these strips were dried thoroughly before using.

(3) The light sensitive coating was exposed through a photographic positive for 6 minutes in the same setup as described in Example I, step 2.

(4) The exposed light sensitive coating was rolled into contact with the image-receiving coating through a bath containing tap water for a period of 5 seconds.

The coatings were then stripped apart 5 to 10 seconds after they had emerged together from the roller system.

It was found that:

- (1) The unexposed letters of the light sensitive coating transferred satisfactorily to the image-receiving layer; very little of the exposed background transferred.
- (2) A reversal image consisting of red-brown letters on a very light-pink background was obtained.

*Example VI*

(1) The light sensitive coating was the same as in Example III, step 1.

(2) The image-receiving layer was prepared by coating the following mixture (40° C.) on baryta subbed paper base:

|                                                               |    |     |
|---------------------------------------------------------------|----|-----|
| 8% surface gel                                                | g  | 49  |
| 8% aq. Saponin                                                | ml | 0.5 |
| ZnO                                                           | g  | 1.0 |
| Mn(OAc) <sub>2</sub> solution (9 g./100 ml. H <sub>2</sub> O) | ml | 2.0 |

(3) The light sensitive coating was exposed through a photographic positive for 5 minutes in the setup described in Example I, step 2.

(4) The exposed light sensitive coating was rolled into contact with the image-receiving coating through a bath containing deionized water for a period of 5 seconds.

The coatings were then stripped apart 0 to 20 seconds after they had emerged together from the roller system.

It was found that:

(1) The length of time that the coatings were left in contact had a great effect on the amount of exposed background which transferred to the image-receiving sheet; the shorter the contact period, the less background transfer.

(2) The unexposed letters transferred satisfactorily to the image-receiving layer.

(3) The reversal image obtained from this transfer consisted of—

- (a) Short contact period: brown-red letters on a white background,
- (b) Longer contact period: brown-red letters on a brown background.

*Example VII*

(1) The light sensitive layer used was the same as that described in Example III, step 1.

(2) The image-receiving layer was prepared by coating the following mixture (40° C.) on baryta subbed paper base:

|                                                               |    |     |
|---------------------------------------------------------------|----|-----|
| 8% surface gel                                                | g  | 49  |
| TiO <sub>2</sub>                                              | g  | 1   |
| 8% Saponin                                                    | ml | 0.5 |
| Mn(OAc) <sub>2</sub> solution (9 g./100 ml. H <sub>2</sub> O) | ml | 2   |

(3) The light sensitive coating was exposed through a photographic positive for 5 minutes in the same setup as described in Example I, step 2.

(4) The exposed light sensitive coating was rolled into contact with the image-receiving coating through a bath containing tap water for a period of 10 seconds.

The coatings were then stripped apart 0 to 20 seconds after they had emerged together from the roller system.

It was found that:

(1) The unexposed letters of the light sensitive layer transferred satisfactorily to the image-receiving coating. The exposed background transferred very little to the image-receiving coating.

(2) A reversal image consisting of red-brown letters on a pinkish background was obtained.

*Example VIII*

(1) The light sensitive coating used is the same as that described in Example III, step 1.

(2) The image-receiving layer consisted of colloidal

zinc sulfide in gelatin (see U.S.P. 2,843,485, Yutzy and Cowden, Example I) prepared in the following manner:

(a) Solution A: 1 g. Na<sub>2</sub>S in 1000 ml. deionized H<sub>2</sub>O. Solution B: 1 g. Zn(NO<sub>3</sub>)<sub>2</sub>·6H<sub>2</sub>O in 1000 ml. deionized H<sub>2</sub>O.

(b) With rapid stirring, 100 ml. of solution B was poured into a solution consisting of 23 ml. of solution A diluted with 157 cc. of deionized H<sub>2</sub>O.

(c) The above mixture was poured quickly (at 40° C.) into a solution of 110 grams of 20% gelatin containing 10 cc. of 7.5% aqueous Saponin at 40° C.

(d) The mixture was held at 40° C. for 15 minutes, then coated at 40° C. on baryta subbed paper base.

(3) The light sensitive coating was exposed through a photographic positive for 5 minutes using the setup described in Example I, step 2.

(4) The exposed light sensitive coating was rolled into contact with the image-receiving coating (which had been dampened with H<sub>2</sub>O) through a bath containing tap water for a period of 5 seconds. The coatings were then stripped apart from 0 to 20 seconds after they had emerged together from the roller system.

It was found that:

(1) The unexposed letters of the light sensitive coating transferred satisfactorily to the image-receiving layer; only very small portions of the exposed background also transferred to the image-receiving sheet.

(2) A reversal image consisting of very stable, dark brown letters on a slightly pink background was obtained.

*Example IX*

(1) The light sensitive coating used is the same as that described in Example III, step 1.

(2) The image-receiving layer was prepared by coating the following mixture (40° C.) on baryta subbed paper base:

|                                                                          |    |     |
|--------------------------------------------------------------------------|----|-----|
| 20% gelatin solution                                                     | g  | 110 |
| Deionized water                                                          | ml | 157 |
| Na <sub>2</sub> S solution (1 g. in 1000 ml. deionized H <sub>2</sub> O) | ml | 23  |
| 7.5% aq. Saponin                                                         | ml | 10  |

(3) The light sensitive coating was exposed through a photographic positive for 5 minutes in the same setup described in Example I, step 2.

(4) The exposed light sensitive coating was rolled into contact with the image-receiving coating through a bath containing tap water over a period of 10 seconds. The coatings were then stripped apart 0 to 20 seconds after they had emerged together from the roller system.

It was found that:

(1) The unexposed letters of the light sensitive coating transferred to the image-receiving layer; extremely small amounts of the unexposed background transferred to the image-receiving coating.

(2) A reversal image consisting of light-brown and very stable letters on a white background was obtained.

*Example X*

(1) The light sensitive coating used is the same as that described in Example III, step 1.

(2) The image-receiving coating was prepared by pulling strips of baryta subbed paper base through a slurry of 2.0 grams of zinc oxide in 200 ml. of deionized water (mixing at 60 volts in a metal cup on a Waring Blender).

(3) The light sensitive coating was exposed through a photographic positive for 5 minutes in the same setup as described in Example I, step 2.

(4) The exposed light sensitive coating was rolled into contact with the image-receiving layer through a bath containing tap water for a period of 2 seconds. The

coatings were stripped apart 0 to 20 seconds after they had emerged together from the roller system.

It was found that:

- (1) The unexposed letters of the light sensitive coating transferred satisfactorily to the image-receiving layer; the exposed background transferred very little to the image-receiving layer.
- (2) A reversal image consisting of brown letters on an even background was obtained.

*Example XI*

- (1) The light sensitive coating was the same as that described in Example III, step 1.

(2) The image-receiving layer was prepared by pulling strips of baryta subbed paper base through a mixture of 2 grams of  $TiO_2$  in 200 ml. of deionized water (mixing at 60 volts in a metal cup on a Waring Blender).

(3) The light sensitive coating was exposed through a photographic positive in the setup described in Example I, step 2.

(4) The exposed light sensitive coating was rolled into contact with the image-receiving layer through a bath containing tap water for a period of 2 seconds.

The coatings were then stripped apart 0 to 20 seconds after they had emerged together from the roller system.

It was found that:

- (1) The unexposed letters of the light sensitive coating transferred very nicely to the image-receiving layer, but little of the exposed background transferred to the image-receiving layer.

(2) A reversal image consisting of brown letters on a pinkish background was obtained.

*Example XII*

- (1) The light sensitive coating was the same as that used in Example III, step 1.

(2) The image-receiving layer was prepared by coating the following mixture (40° C.) on baryta subbed paper base:

Colloidal zinc sulfide (see Example VIII, step 2) \_\_\_\_\_ ml. 50

Ascorbic acid \_\_\_\_\_ g. 1

10% aqueous K-Cr-Alum \_\_\_\_\_ ml. 0.5

$TiO_2$  \_\_\_\_\_ g. 0.5

(3) The light sensitive coating was exposed through a photographic positive for 5 minutes in the setup described in Example I, step 2.

(4) The exposed light sensitive coating was rolled into contact with the image-receiving coating through a bath containing tap water for a period of 5 seconds.

The coatings were stripped apart from 0 to 20 seconds after they had emerged together from the roller system.

It was found that:

- (1) The unexposed letters of the light sensitive layer transferred satisfactorily to the image-receiving layer; none of the exposed background transferred.

(2) A reversal image consisting of brown stable letters on a white background was obtained.

*Example XIII*

- (1) The light sensitive layer was the same as that described in Example III, step 1.

(2) The image-receiving layer was prepared by pulling strips of baryta subbed paper base through a solution consisting of

Silica powder (Floated Powder, 240 mesh, Fisher,

Catalog No. S-153) \_\_\_\_\_ g. 0.5

Deionized water \_\_\_\_\_ ml. 100

Ascorbic acid \_\_\_\_\_ g. 1.0

(3) The light sensitive layer was exposed through a photographic positive for 4 minutes in the setup described in Example I, step 2.

(4) The exposed light sensitive coating was rolled into contact with the image-receiving coating through a bath containing tap water for a period of 10 seconds.

The coatings were then stripped apart 5 seconds after they had emerged together from the roller system.

It was found that:

- (1) The unexposed letters of the light sensitive layer transferred to the image-receiving layer; the exposed background did not transfer.

(2) A reversal image consisting of brown-black letters on a white background was obtained.

*Example XIV*

- (1) The light sensitive layer was the same as in Example III, step 1.

(2) The image-receiving layer was prepared by pulling strips of baryta subbed paper base through a mixture of

20 0.1% aqueous  $Zn(NO_3)_2 \cdot 6H_2O$  solution \_\_\_\_\_ ml. 100

0.1% aqueous  $Na_2S$  solution \_\_\_\_\_ ml. 23

Deionized water \_\_\_\_\_ ml. 157

Ascorbic acid \_\_\_\_\_ g. 1.0

Silica (Floated Powder—240 Mesh, Fisher, Cata-

25 log No. S-153) \_\_\_\_\_ g. 0.5

(3) The light sensitive coating was exposed through a photographic positive for 6 minutes in the setup described in Example I, step 2.

(4) The exposed light sensitive coating was rolled into contact with the dampened image-receiving coating through a bath containing tap water for a period of 2 seconds.

The two layers were stripped apart 0 to 20 seconds after they had emerged together from the roller system.

It was found that:

- (1) The unexposed letters of the light sensitive coating transferred to the image-receiving layer, the exposed background transferred also a little to the image-receiving coating.

(2) A reversal image consisting of brown letters on a grey-white background was obtained.

*Example XV*

- (1) The light sensitive coating used is described in Example III, step 1.

(2) The image-receiving coating was prepared by pulling strips of baryta subbed paper base through a mixture of sensitizing dye of the following composition:

50 3,3'-diethyl-9-methylthiacarbocyanine iodide



55 (25 mg./250 ml. methanol) \_\_\_\_\_ ml. 0.25

Deionized water \_\_\_\_\_ ml. 100

60 Ascorbic acid \_\_\_\_\_ g. 1.0

Silica (same as Example XIV, step 2) \_\_\_\_\_ g. 0.5

(3) The light sensitive coating was exposed through a photographic positive for a period of 5 minutes in the setup described in Example I, step 2.

(4) The exposed light sensitive coating was rolled into contact with the image-receiving coating through a bath containing tap water for a period of 2 seconds.

The coatings were stripped apart from 0 to 20 seconds after they had emerged together from the roller system.

It was found that:

- (1) The unexposed letters of the light sensitive coating transferred to the image-receiving coating; some of the exposed background transferred also.

(2) A reversal image consisting of brown letters on a pink-brown background was obtained.

*Example XVI*

(1) The light sensitive coating was the same as that described in Example III, step 1.

(2) The image-receiving coating was prepared by coating the following mixture (at 40° C.) on baryta subbed paper base:

|                                                                                                                                                              |     |
|--------------------------------------------------------------------------------------------------------------------------------------------------------------|-----|
| A suspension of colloidal silver in gelatin (with 9 g. of colloidal silver per kg. of suspension and particle sizes of 20-30 millimicrons diameters) ---g--- | 5   |
| 6% surface gel-----ml.                                                                                                                                       | 35  |
| 10% aqueous K-Cr-Alum-----ml.                                                                                                                                | 1   |
| Ascorbic acid-----g.                                                                                                                                         | 1   |
| 8% Saponin-----ml.                                                                                                                                           | 0.3 |

(3) The light sensitive layer was exposed through a photographic positive for 5 minutes in the same setup as described in Example I, step 2.

(4) The actual image transfer was made as follows: The exposed light sensitive coating was rolled into contact with the dampened image-receiving coating through a bath containing tap water for a period of 2 seconds.

The coatings were then stripped apart 5 seconds after they had emerged together from the roller system.

It was found that:

- (1) The unexposed letters transferred very satisfactorily to the image-receiving layer; no background transfer took place.
- (2) A reversal image consisting of very stable, black letters on yellow background was obtained.

*Example XVII*

(1) The light sensitive coating was prepared as follows:

|                                       |     |     |
|---------------------------------------|-----|-----|
| 6% aq. surface gel-----               | 40  | ML. |
| Aq. AgNO <sub>3</sub> solution A----- | 5   |     |
| Water-----                            | 3   |     |
| Ammonium citrate solution B-----      | 1   |     |
| 10% aq. Potassium Chrom Alum-----     | 2   |     |
| 8% aq. Saponin-----                   | 0.5 |     |

The above mixture was coated on subbed film base and paper.

- (A) 0.850 g. AgNO<sub>3</sub> per 5 ml. volume
- (B) Mix the following ingredients:

|                             |     |      |
|-----------------------------|-----|------|
| Water-----                  | ml. | 50.0 |
| Citric acid-----            | g.  | 12.0 |
| 28% NH <sub>4</sub> OH----- | ml. | 12.0 |

slowly, with stirring and cooling. Ref.: Phot. Eng., 5, 127 (1954).

(2) The image-receiving coating was prepared by coating the following mixture at 40° C. on subbed film base and paper:

|                                                      |     |      |
|------------------------------------------------------|-----|------|
| Yellow Filter Noodles (same as in Example XVI) ----- | g.  | 0.05 |
| 6% aq. surface gel-----                              | ml. | 50.0 |
| 10% aq. Potassium Chrom Alum-----                    | ml. | 1.0  |
| Ascorbic acid-----g.                                 |     | 1.0  |
| 8% aq. Saponin-----ml.                               |     | 0.5  |

(3) The light sensitive layer was exposed through a photographic positive for 5 minutes in the same setup as described in Example I, step 2.

(4) The actual image transfer was made as follows:

The exposed light sensitive coating was rolled into contact with the dampened image-receiving layer through a bath containing tap water for a period of 2 seconds.

The coatings were then stripped apart 4 seconds after they had emerged together from the roller system.

It was found that:

- (1) The unexposed letters transferred very satisfactorily to the image-receiving layer; no background took place.

- (2) An almost completely dry reversal image consisting of very stable, black letters on a light yellowish background was obtained.
- (3) It was found that the final image can be stored for long periods of time without deleterious effects.

The apparatus used in pressing together the light sensitive layer and the image-receiving layer may be of very simple construction. Thus, one of the layers may be wetted with water and the two layers pressed together by running over them with a rubber roller. The two layers are then separated and dried. The image appears on the image-receiving layer. The two layers may also be placed into a Constat or Ozalid Photo Copy Processor machine. This machine is nothing more than a rubber roller system mounted in a tray. In operation, the tray is filled with water and the handle turned which causes the two rollers to rotate at the same speed resulting in the two layers being pressed together.

Modifications will appear to persons skilled in the art. I, therefore, do not intend to be limited in the patent granted except as necessitated by the appended claims.

I claim:

1. A process of forming a positive silver image in an image receiving layer which comprises imagewise exposing a silver salt print-out emulsion layer containing a water-soluble silver salt so as to form metallic silver in the exposed areas of said print-out layer and then contacting said exposed silver salt emulsion layer under pressure with said image receiving layer in the presence of pure water, whereby said water-soluble silver salt in the unexposed portions of the emulsion is dissolved in said pure water, transferred to the receiving layer and converted into metallic silver in the presence of a nucleating agent for promoting image formation which is located in said image receiving layer, thereby transforming the dissolved silver salt which is transferred and deposited in said receiving layer into a visible image.

2. A process according to claim 1 wherein said nucleating agent is a chemical precipitant.

3. A process according to claim 1 wherein said nucleating agent for promoting image formation comprises physical development nuclei.

4. A process of forming a positive silver image in an image receiving layer comprising a baryta subbed paper having a coating comprising phenyl-mercapto-tetrazole thereon, which comprises exposing imagewise, a silver chloride print-out emulsion layer containing an excess of silver nitrate so as to form metallic silver in the exposed areas of said print-out layer and then contacting said exposed silver chloride print-out emulsion under pressure with said image receiving layer in the presence of pure water which is used as the sole processing agent, thereby dissolving the silver nitrate in the unexposed portions of the print-out emulsion and transferring it to the receiving layers where said dissolved water-soluble silver salt is deposited as metallic silver in visible form.

5. A process as recited in claim 1 wherein the soluble silver salt is silver nitrate.

6. A process as recited in claim 1 wherein the soluble silver salt is silver citrate.

7. A process as recited in claim 1 wherein the print-out emulsion also contains silver chloride as the silver salt.

8. A process as recited in claim 1 wherein the image-receiving layer comprises baryta subbed paper.

9. A process as recited in claim 1 wherein the image-receiving layer comprises baryta subbed paper having a coating thereon comprising MnSO<sub>4</sub>.

10. A process as recited in claim 1 wherein the image-receiving layer comprises baryta subbed paper having a coating thereon comprising ascorbic acid.

11. A process as recited in claim 1 wherein the image-receiving layer comprises baryta subbed paper having a coating thereon comprising phenyl-mercapto-tetrazole.

12. A process as recited in claim 1 wherein the image-receiving layer comprises baryta subbed paper having a coating thereon comprising  $ZnO$ .

13. A process as recited in claim 1 wherein the image-receiving layer comprises baryta subbed paper having a coating thereon comprising  $Mn(OAc)_2$ .

14. A process as recited in claim 1 wherein the image-receiving layer comprises baryta subbed paper having a coating thereon comprising  $TiO_2$ .

15. A process as recited in claim 1 wherein the image-receiving layer comprises baryta subbed paper having a coating thereon comprising  $Na_2S$ .

16. A process as recited in claim 1 wherein the image-receiving layer comprises baryta subbed paper having a coating thereon comprising  $Zn(NO_3)_2$ .

17. A process as recited in claim 1 wherein the image-receiving layer comprises baryta subbed paper having a coating thereon comprising  $ZnS$ .

18. A process as recited in claim 1 wherein the image-receiving layer comprises baryta subbed paper having a coating thereon comprising Silica in finely dispersed form.

19. A process as recited in claim 1 wherein the image-receiving layer comprises baryta subbed paper having a coating thereon comprising colloidal silver.

20. A process as recited in claim 1 wherein the image-receiving layer comprises 2-mercaptopbenzothiazole.

21. A process as recited in claim 1 wherein the moisture is supplied by means of tap water.

22. A process as recited in claim 1 wherein the moisture is supplied by means of deionized water.

23. A process as recited in claim 1 wherein the moisture is supplied by means of steam.

References Cited in the file of this patent

UNITED STATES PATENTS

15 2,846,309 Land \_\_\_\_\_ Aug. 5, 1958

FOREIGN PATENTS

566,522 Canada \_\_\_\_\_ Nov. 25, 1958

695,905 Great Britain \_\_\_\_\_ Aug. 19, 1953

OTHER REFERENCES

Dybvig et al.: Photographic Engineering, vol. 5, No. 2, pp. 127-132 (1954).